

Feb. 7, 1939.

J. H. DE BOER ET AL

2,146,099

SECONDARY ELECTRON EMMITTER AND METHOD OF MAKING IT

Filed May 21, 1937

*Fig. 1*



*Fig. 2*



INVENTORS

JAN HENDRIK DE BOER,  
HAJO BRUINING,  
FRITS PRAKKE AND  
KAREL MARINUS VAN GESSEL

BY

*Charles McClair*  
ATTORNEY.

## UNITED STATES PATENT OFFICE

2,146,099

SECONDARY ELECTRON Emitter AND  
METHOD OF MAKING IT

Jan Hendrik de Boer, Hajo Bruining, Frits Prakke,  
and Karel Marinus Van Gessel, Eindhoven,  
Netherlands, assignors to N. V. Philips' Gloeilampenfabrieken, Eindhoven, Netherlands

Application May 21, 1937, Serial No. 143,946  
In Germany February 10, 1936

5 Claims. (Cl. 250—174)

This invention relates to a surface having a high secondary electron emitting capacity and to a method of manufacturing such a surface.

Although it is generally sought to reduce to a minimum the secondary emission of the electrodes of an electric discharge tube, for instance of the grids and the anodes, there are cases in which it is just electrodes having a high secondary emission that are wanted, for example, in electron amplifying tubes, the so-called "electron multipliers", in which a very high amplification is sought to obtain.

For achieving a high secondary emission it is known to furnish surfaces with a layer of caesium oxide and caesium absorbed thereon, which layer is sometimes mixed with other oxides or metal particles and may also contain caesium. However, such a layer can be prepared inside the tube only and its preparation requires many operations so that the risk of failure is comparatively great.

We have now devised a surface which has a very high secondary emission and can be established in a very simple manner, while the preparation need not be effected inside the tube, but can be carried out by a separate operation, the surface being afterwards introduced into discharge tubes and the like. A surface according to the invention consists of a pure carbon layer having a high adsorption power and having adsorbed to it one or more metals of the second principal group of the periodic system having an atom number above 4.

A surface according to the present invention may be established, for instance, by coating a supporting body or electrode for example, of nickel with a carbon layer and by applying on to said layer one or more of the metals referred to. Particularly good results are achieved when heating a metal surface in an atmosphere of a simple hydrocarbon, preferably acetylene, in a high frequency member. Thus, by decomposition of the hydrocarbon a pure carbon layer is formed on the metal surface, which layer inherently adsorbs alkaline earth metals. According to the invention one or more of the above-mentioned metals are then caused to be adsorbed from the vapour-phase by such a layer.

According to one very favorable method according to the invention a supporting body such as a nickel electrode is coated with a layer consisting of one or more oxides or hydroxides of these metals, preferably with magnesium oxide, whereon carbon is precipitated by high frequency heating in an atmosphere consisting of a simple

hydrocarbon, the body thus obtained being subsequently heated for some time in a high vacuum. The hydrocarbons may, for instance, be acetylene, methane or the like. The heating operation after provision of the carbon may, for instance, be effected at a temperature of 900 to 1000° C. Very probably the oxide is partly reduced thereby and the metal produced is adsorbed to the carbon.

Owing to the easy method of manufacture, surfaces according to the present invention may advantageously be used in electric discharge tubes, more particularly in so-called "electron multipliers".

It has been found that such a surface may have a very high secondary emission which in many cases may be of the order of magnitude of 5 secondary electrodes per primary electron.

The method according to the invention may be carried out as follows.

A nickel electrode is coated with a layer of magnesium oxide, which may be effected, for instance, by spraying. An electrode thus coated is introduced into an acetylene atmosphere and then the electrode is covered with a carbon layer by high frequency heating. This treatment may, for instance, take several minutes. After that the electrode together with other parts is introduced into the bulb of a discharge tube and then the tube is exhausted. After that the surface obtained is heated, for some moments to a temperature of about 900° C. which may also be effected by high frequency heating. It has been found that a surface thus established permits a secondary emission to be obtained of the order of magnitude of 6 secondary electrons per primary electron at a voltage of 500 volts.

In the accompanying drawing Figure 1 shows the steps of the method according to the invention, and Figure 2 shows in greatly enlarged cross-section a portion of an electrode made in accordance with the invention.

In Figure 1 the outer rectangles numbered 1, 2, 3, and 4 represent the successive steps of the method, rectangles 2 and 4 representing steps which are always used. The small rectangles inside rectangles 1 and 3 represent alternative ways of carrying out the first and third steps. If, in step 1 the alternative a is adopted, and the core is clean or uncoated nickel, then in step 3 the alternative a of exposure to magnesium vapor is followed. If, in step 1 the alternative b is adopted, and the core is nickel with a magnesia coating, then in step 3 the alternative b of proceeding directly to the final step is followed.

The final step, represented by the large rectangle 4, is used regardless of which alternative *a* or *b* is adopted in preceding steps 1 and 3.

The finished electrode shown in Figure 2 comprises a nickel core 5 on which is a layer 6 of pure carbon deposited on the core by high frequency induction heating in an atmosphere of simple hydrocarbon, such as acetylene. The pure carbon layer contains or is impregnated with an alkaline earth metal such as magnesium absorbed in the carbon layer as indicated by the small crosses 7, and supplied to the carbon layer by exposure to vaporized magnesium, or by reduction of the magnesia on the magnesia coated core by the carbon.

What we claim is:

1. The method of making a surface having secondary electron emissivity several times unity which consists in coating a metal core body with a coating of carbon by heating said body by high frequency induction heating in an atmosphere of a simple hydrocarbon, metallizing the surface of said coated body by depositing on it an alkaline earth metal from the vapor-phase, and then heating the metallized body in vacuum.
2. The method of making a surface having secondary electron emissivity several times unity which consists in coating a metal core body with a layer of carbon absorbent of alkaline earth metal by heating said body by high frequency induction to a high temperature in an atmosphere of acetylene at substantially room temperature, exposing said carbon coated body in vacuum to an excess of vapor of an alkaline earth metal to cause metal from the vapor-phase to be adsorbed by said carbon coated body, and then heating said body by high frequency induction heating to about 900° C.

3. The method of producing an electrode having secondary electron emissivity several times unity which comprises coating a body of nickel with carbon highly absorbent of alkaline earth metal by heating said body to a high temperature in an atmosphere of acetylene by high frequency induction heating, treating said carbon coated body at room temperature with an excess of magnesium vapor to impregnate said carbon with magnesium, and heating said body in vacuum at about 900° C. for several minutes to activate said electrode.

4. The method of producing an electrode having secondary electron emissivity several times unity which comprises coating a body of nickel with magnesium oxide, producing on said coated body a layer of carbon highly absorbent of alkaline earth metal by heating said body to a high temperature in an atmosphere of acetylene by high frequency induction heating, and heating said body in vacuum at about 900° C. for several minutes to activate said electrode.

5. A secondary electron emitting electrode having a ratio of secondary electron emission of several times unity upon impact by primary electrons at several hundred volts which comprises a metal core, a layer of alkaline earth oxide on and adherent to said core, and a pure carbon coating on and in contact with said layer and having the alkaline earth metal of said layer absorbed in said carbon.

JAN HENDRIK DE BOER.

HAJO BRUINING.

FRITS PRAKKE.

KAREL MARINUS VAN GESSEL.

35